

July 29, 1947.

M. C. JAY

2,424,931

METAL MOLD

Filed Dec. 26, 1942



INVENTOR:  
MATTHEW C. JAY,  
BY: *John E. Jackson*  
HIS ATTORNEY.

Patented July 29, 1947

2,424,931

# UNITED STATES PATENT OFFICE

2,424,931

## METAL MOLD

Matthew C. Jay, Gary, Ind.

Application December 26, 1942, Serial No. 470,255

2 Claims. (Cl. 22—188)

1

This invention relates to improvements in metal molds for casting metal at high temperatures.

Molds for casting test pieces or specimens of heats of steel have been employed heretofore made of what is generally termed Swedish steel, the prime requisites of such a mold being the repeated casting of specimens of uniform dimension at high temperatures of from 2600° F. to 3200° F. without fusion with the mold. While such prior molds have been successfully employed, their span of life is too short; they suffer rapid oxidation; frequently become spotted by alloy metals; and do not permit of water quenching for quick cooling.

It is a prime object of my invention to provide a mold of the character stated composed of a metal which will obviate the objections heretofore stated, and which may be produced and used with a considerable saving in cost.

Additional objects and advantages will become apparent from the following description taken in connection with the accompanying drawing which illustrates a mold of the character referred to and embodying the present invention.

As illustrated, the mold may comprise halves or separable complementary sections A, each having an elongate half-cylindrical mold cavity 2 combining to mold a test piece of cast metal of a desired length and cross sectional area to serve in resistance testing for carbon content in suitable apparatus generally employed in the art for such test. The cavities 2 have complementary sprue portions 3 extending to one outer face of the mold to receive the molten metal.

The mold A is machined to substantially the size and contour, formerly employed for such molds, from a killed i. e., substantially completely deoxidized, steel containing not more than 0.12 carbon and not more than 0.25 copper. I have found the following compositions and range to produce satisfactory results:

|                 | Example I | Example II | Range           |
|-----------------|-----------|------------|-----------------|
| Carbon.....     | 0.12      | 0.11       | 0.05 to 0.12    |
| Manganese.....  | 0.40      | 0.40       | 0.30 to 0.60    |
| Phosphorus..... | 0.010     | 0.10       | to 0.10 maximum |
| Sulphur.....    | 0.037     | 0.037      | to 0.04 maximum |
| Silicon.....    | 0.08      | 0.08       | 0.10 and under  |
| Copper.....     | 0.24      | 0.24       | 0.25 and under  |
| Nickel.....     | 0.03      | 0.03       |                 |

the balance being substantially pure iron, except for impurities. Such steel may be killed by common deoxidizing agents with satisfactory results so long as the end product contains carbon and copper within the specified range above.

2

A mold having the foregoing composition possesses the ability to withstand high temperatures within the range stated without fusion with the molten metal. Consecutive test specimens of both basic and acid high and low carbon steels were successfully cast in such a mold at temperatures up to 3000° F., each cast being followed by quenching of the mold in water.

The metal from which the mold is formed is sufficiently soft to be readily machined, and undergoes minimum oxidation, even despite the water quenching, thereby preventing injury to the cast specimens, as by spotting. The life of such a mold in service has been found to be more than three times that of the former Swedish steel molds, and may be produced at considerably lower cost.

Various changes and modifications are contemplated within the scope of the following claims.

20 I claim:

1. A test mold for casting metal test pieces composed of a killed low carbon steel containing copper in effective amounts but not exceeding 0.25, said mold having the characteristics of preventing fusion with the molten metal cast therein at temperatures up to substantially 3000° F., and of effectively resisting spotting upon subsequently being quenched in water.

30 2. A test mold for casting metal test pieces composed of a killed low carbon steel containing from about 0.05 to 0.12 carbon, 0.30 to 0.60 manganese, copper in effective amounts but not exceeding 0.25, phosphorus not to exceed 0.10, sulphur not to exceed 0.04, silicon not to exceed 0.10, with the balance being substantially pure iron, said mold having the characteristics of preventing fusion with the molten metal cast therein at temperatures up to substantially 3000° F., and of effectively resisting spotting upon subsequently being quenched in water.

MATTHEW C. JAY.

## REFERENCES CITED

45 The following references are of record in the file of this patent:

## UNITED STATES PATENTS

| Number       | Name     | Date          |
|--------------|----------|---------------|
| 50 1,191,473 | Robinson | July 18, 1916 |
| 2,132,276    | Spalding | Oct. 4, 1938  |

## OTHER REFERENCES

55 Alloys of Iron and Copper, by Gregg and Daniloff, page 222. Published by Maple Press Co., 1934, York, Pa.